

## 1

3,127,353

### LUBRICATING COMPOSITIONS

Ernst Roos, Leverkusen, Friedrich Lober, Leverkusen-Bayerwerk, and Walther Lohmar, Mülheim (Ruhr), Germany, assignors to Farbenfabriken Bayer Aktiengesellschaft, Leverkusen, Germany, a corporation of Germany

No Drawing. Filed July 10, 1959, Ser. No. 826,124  
4 Claims. (Cl. 252—52)

The present invention relates to lubricating compositions; more particularly it concerns lubricating compositions containing a lubricant, especially a lubricant based on mineral oils, and an aryl-glycide ether of the general formula



wherein R stands for an alkyl radical containing at least 12 carbon atoms.

Suitable aryl-glycide ethers are for instance 4-dodecyl-phenoxy-propene oxide, 4-isododecyl-phenoxy-propene oxide, 3-pentadecyl-phenoxy-propene oxide, 4-octadecyl-phenoxy-propene oxide and 4-isoctadecyl-phenoxy-propene oxide.

Aryl-glycide ethers of this type are obtainable by various methods, e.g. by reacting epichorohydrin with phenols which are substituted by an alkyl radical containing at least 12 carbon atoms, or by epoxylating the corresponding arylallyl ethers; in general, they are viscous, colourless or slightly coloured, odourless liquids.

The aryl-glycide ethers present in the lubricating compositions of the invention increase mainly the thermal stability of the lubricants to which they impart good high-pressure properties as well as detergent action; moreover, it is remarkable that they are compatible with other lubricant additives such as antioxidants or anti-corrosion agents. The requisite quantities of aryl-glycide ethers may readily be established by preliminary experiments; in general, an addition of 0.1 to 5 percent by weight, referred to the lubricant, is sufficient.

It is already known to add to lubricants aryl-glycide ethers of the general formula



wherein Ar stands for a phenyl radical which is not substituted or which is only substituted by alkyl radicals containing on the whole at most 4 carbon atoms. Compared with such additives the aryl-glycide ethers of the present invention are surprisingly more active. This can be seen from the following table concerning relevant tests. The evaluation data were obtained by subjecting mixtures of 100 parts by weight of a naphthenic oil SAE 20 and 2 parts by weight of one of the aryl-glycide ethers indicated for 50 hours in a one-cylinder-four-stroke

## 2

MWM-diesel engine to a test such as has been described in "Erdöl und Kohle" 12, pages 484—489.

Table

|    | Aryl-glycide ether | Evaluation note |
|----|--------------------|-----------------|
| 5  |                    | 66              |
| 10 |                    | 63              |
| 15 |                    | 68              |
| 20 |                    | 81              |
| 25 |                    | 77              |
| 30 |                    | 76              |

We claim:

35 1. A lubricating composition comprising a major amount of a lubricant and 0.1—5% by weight of an aryl-glycide ether of the general formula



wherein R stands for an alkyl radical containing at least 12 carbon atoms.

40 2. A lubricating composition comprising a major amount of a mineral oil lubricant and 0.1—5% by weight of 4-isododecyl-phenoxy-propene oxide.

45 3. A lubricating composition comprising a major amount of a mineral oil lubricant and 0.1—5% by weight of a 3-pentadecyl-phenoxy-propene oxide.

50 4. A lubricating composition comprising a major amount of a mineral oil lubricant and 0.1—5% by weight of an 4-octadecyl-phenoxy-propene oxide.

### References Cited in the file of this patent

### UNITED STATES PATENTS

2,665,254 Coppock \_\_\_\_\_ Jan. 5, 1954